

Dec. 1, 1942.

O. R. SCHULTZ ET AL

2,303,395

METHOD OF MAKING DECORATED MATERIAL

Filed April 20, 1939



Fig. 1



Fig. 2



Fig. 3



Fig. 4



Fig. 5



Fig. 6



Fig. 7



Fig. 8



Fig. 9



INVENTORS  
3 Osvald R. Schultz  
BY Henry D. Tucker  
Aubra J. Carlson  
ATTORNEY

## UNITED STATES PATENT OFFICE

2,303,395

## METHOD OF MAKING DECORATED MATERIAL

Oswald R. Schultz, New York, N. Y., and Henry D. Tucker, Rahway, N. J., assignors to Cellu-Type Plate Company, Incorporated, New York, N. Y., a corporation of New York

Application April 20, 1939, Serial No. 268,914

5 Claims. (Cl. 41—25)

This invention relates to decorated material and method of making same, and is particularly concerned with material suited for such constructional and decorative purposes as wallboard, paneling, table tops, counters, wall covering, etc. The products resulting from the processes of the invention are distinguishable not only by their excellent wearing qualities and resistance to soiling and defacement, but by their distinctive ornamental appearance. The ornamental character of the products of the invention is greatly enhanced by the embossed and colored designs obtainable by the application of the principles of the process.

Objects of the invention are to produce constructional and decorative material having these properties in a simple and economical manner without the use of thermoplastics, the carefully etched metal dies, and the costly heat and pressure equipment required thereby. Furthermore, the invention permits continuity of operation, which is of distinct commercial advantage.

Another object is to produce unique decorative designs, plain, embossed or in color, on composition board, paper, cloth or other material adapted to receive the same.

Other objects will more clearly appear as we proceed with the description of the invention.

The materials from which the desirable surfacing is obtained and with which the invention is especially concerned are synthetic resins of the cold plasticizable or cold moldable type, and which have hardening accelerators incorporated therein. These are well adapted to acquire ornamental impressions when processed according to the present invention, and when solidified and related to a suitable foundation produce the unique and valuable commercial products herein described.

Cold plasticizable resins of this type can be molded substantially at room temperature and upon solidification and hardening maintain and preserve the design or impression molded therein. We may use phenolic resin formed by compounding carbolic acid or phenol and formaldehyde such as is commercially available in the form of a solvent-containing viscous liquid or semi-solid. We may also use derivatives of urea, either alone or in combination with such phenol and resins. The material may have incorporated therein various fillers or other suitable material, but for best ornamental results should have coloring ingredients included therein, as will be hereinafter explained. As an example of one type of such material that is suited for use in accordance with

the invention, we may mention the viscous liquid obtainable from the phenolic resin known by the trade name "Catalin."

In order to produce the novel products of the invention, we adopt novel molding equipment and procedure. We have discovered that cold set acidified phenolic resin in the viscous liquid or semi-solid state will not mold readily from ordinary metal surfaces, such as copper, aluminum or ferrous metals, due to the fact that the acid in such resins reacts with the metal and creates bubbles of gas which cause undesirable blisters and irregularities in the molded surface. To obviate this difficulty we form the molding matrix from a material which does not produce these undesirable effects, so that the molded product will be free from undesirable deformations and so that the finished surface will carry the desired pattern in accurate relief. Matrices suited for these purposes may be made in various ways but they are all characterized by the presence of an embossing surface composed of a cellulose derivative such as cellulose nitrate or acetate, which surface has no considerable affinity or reactive capacity for cold moldable resins of the type described and which may easily be stripped therefrom.

Briefly described, the process of the invention comprises providing a suitable foundation or backing, spreading a viscous solution of a cold moldable resin in a suitable solvent upon the backing, rolling the cellulose covered embossed matrix over the applied resin under a pressure which in contradistinction to those used in hot plate methods is only sufficient firmly and evenly to press the matrix into the resin, so that the resin is sandwiched between the matrix and the backing. The process proceeds by allowing the resin to set either by allowing it to stand at room temperatures for a suitable time or by placing the assembly in an oven in order to allow the accelerating ingredients to function and the solvent to be driven off more rapidly. The coating is thus very intimately associated with the backing in the form of an integral structure and the matrix is easily stripped therefrom.

The matrix with which the cold moldable plastic is embossed may be prepared in a number of different ways. It may be prepared by transferring the embossed design of a water-swollen gelatinous compound to a backing coated with a cellulose derivative as described in the patent to Schultz No. 2,085,048, dated June 29, 1937. It may be prepared by coating an etched metal plate with cellulose and using the coated member as a ma-

trix. It may be prepared by transferring the design of an etched metal plate or roller to a somewhat flexible backing by applying a suitable cellulosic or gelatinous "dope" between the plate and the backing, subjecting the assembly to pressure, and then stripping the thus embossed backing from the plate or roller and utilizing the stripped member as a matrix. Or it may be prepared by coating any embossed design, which we shall call a copy relief, with a layer of cellulose nitrate or acetate and transferring the layer, which acquires the same design as the copy relief, by pressure onto a substantially non-stretchable backing in order to reproduce the design on the backing, drying the combined copy relief and the doped backing and then stripping off the copy relief. It may be obtained without any preparation whatever by utilizing ordinary fabric or fibrous material coated with cellulose compounds and provided with an embossed design thereon.

Furthermore, the matrix instead of being embossed may be taken from a perfectly smooth, and flat surface, with the result that the surface of the applied resin takes on the exact counterpart of this smooth flat surface. This is of distinct advantage in producing perfectly smooth flat surfaces with simplicity and economy.

In choosing a backing for whatever matrix is desired, it is preferable to use a fabric backing covered with a prepared somewhat flexible cellulose compound, as this is of considerable advantage over a straight nitrocellulose sheet which is likely to be stiff and unmanageable and which is a constant fire hazard. Fabrics like those known commercially as "Permatex," "Fabrikoid" and "Karatol" are satisfactory for this purpose.

It should be noted that regardless of the way the matrix is formed, the same consists of an embossed design or a flat surface preferably on a somewhat flexible backing, the surface carrying a thin film of cellulosic or gelatinous material which has no affinity for, nor any undesirable effect upon the synthetic resins with which the invention is concerned. Such matrices may be easily stripped from the applied resinous coating after the same has set, and may be used over and over again.

The invention will be more clearly understood when reference is had to the accompanying drawing in which the process and product are shown diagrammatically. The thicknesses of the coatings illustrated are of course greatly enlarged for facility of explanation.

Fig. 1 is a view of a backing being spread with a resinous coating;

Fig. 2 represents an elevation of a coated backing with a matrix prepared in accordance with the invention being rolled thereon;

Fig. 3 shows the backing with the matrix pressed into intimate contact therewith;

Fig. 4 shows the matrix being stripped off the backing;

Fig. 5 illustrates how a colored layer of resinous material may be spread on a matrix;

Fig. 6 shows how this colored layer may be applied to a backing to which a different colored coating of resin has been applied;

Fig. 7 shows how the matrix may be stripped from the backing after the top colored layer has adhered to the bottom layer and partially dried thereon, leaving a multi-colored embossed pattern thereon;

Fig. 8 illustrates a modified way of producing a multi-colored design;

Fig. 9 is a fragmentary plan view of a coating, like that shown in Fig. 8; and

Fig. 10 is an elevational diagrammatic view of one way in which the process may be carried out continuously.

Similar reference characters refer to similar parts throughout the various views of the drawing and the specification.

A simple embossed design may be applied to a suitable backing as indicated in Figs. 1 to 3. A layer of cold moldable resinous material 3 is applied by doctor blade 2 on a backing 1, as indicated in Fig. 1. The result is that the backing is covered with a thin smooth even layer of cold moldable resin. The matrix may then be applied on top of this layer, as by slowly rolling matrix 8 having an embossed design set out in relief by indentations 6 over the top of the layer 3 by means of roller 4. The roller 4 is preferably moved slowly from one end of the plate to the other in order to avoid entrapping air beneath the matrix and in order accurately to reproduce the embossed design. After this is accomplished the assembly takes the form shown in Fig. 3 with the matrix pressed in intimate contact with the plasticizable resin and leaving the exact counterpart of design 6 on the top of layer 3, which is very intimately secured and adhered to backing 1. The coated member may then be put into an oven and dried at such temperatures as will cause hardening of the resin and drive off whatever volatile solvents have been incorporated therein. The matrix may now be stripped as indicated in Fig. 4.

In Figs. 5 and 7 we have endeavored to show how a multi-colored embossed design may be obtained. A coated cloth backing 10 provided with indentations 11 representing the desired design is spread with a cold moldable resinous composition 12 by doctor blade 13 so that the composition is retained in the indentations. These indentations, of course, represent an embossed surface which has been impressed upon a cellulose coating in the manner previously described. The resinous coating thus applied is of a color that will contrast with a subsequent colored coating later to be applied to the backing. The matrix having the colored resin 12 contained in its indentations should now be allowed to set.

After this, a layer of resin of a different color is applied in a thin layer to the backing 1, as indicated at 3 in Fig. 6. The matrix previously described, containing the set color 12, is then rolled under a roller 14 so that it is pressed in intimate engagement with the layer 3, and so that the color 12 in the interstices of the matrix is firmly pressed and adhered into the layer 3. The assembly thus formed may then be conveyed to an oven where it may be left a sufficient time to allow the coatings to dry sufficiently so that the matrix may be stripped from the applied coating as indicated in Fig. 7. After the matrix is stripped the finished article is obtained in the form of an embossed design of color 12 outlined over differently colored layer 3, which gives a very pleasing effect.

In Figs. 8 and 9 we have shown another way of obtaining a multi-colored coating. A transparent coating 16 of resin is first applied to a colored base 1. An embossed design 12 of a different color is then applied to the backing 1 in the manner indicated in connection with the description of Figs. 5, 6, and 7, so that the portions 12 of the second color are applied thereon. After the assembly has dried and set, the matrix which carried the second color is stripped off, giving a

design 12 of one color laid on a background 16 of another color.

In Fig. 10 we have shown one way in which the process may be carried out continuously. A sheet 20 of material such as paper, which is adapted to receive and hold the desired embossed design, is run through a pair of embossing rollers 21 carrying design 19, and then subjected to one or more sprays 22 of cellulosic material in order to put a thin coating on the embossed design and to stiffen the paper somewhat. This is dried by driving out the solvents in an oven 23 through which the sheet 20 is continuously carried. The sheet, which is now a matrix with the coated and embossed design 19 thereon is then passed over idler 24 and applicator roll 25 which presses the matrix into a body 3 of cold moldable resin which has been applied on a backing 1 by stationary doctor blade 32 as the backing travels thereunder. The backing is carried along at the same surface speed as roller 25 by conveyor 28. The combined matrix, resin and backing is then carried through oven 30 at the end of which a roller 29 strips the embossed paper 20 from the dried and set coating 3 and the coated and embossed backing is delivered continuously at 31.

It should, of course, be understood that the cold moldable resinous compound required for use in the process contains hydrochloric, phosphoric, or other acidic or hardening compounds in order that relatively rapid hardening, whether or not accelerated by heat, may be accomplished. It is important, therefore, to adjust the pH of the resinous composition so that setting may be accomplished within commercially practicable times. While the time required for setting will vary according to the acidity of the composition, the temperature of the oven and other factors, it is generally expedient that setting times not extend over a period of more than one hour.

Temperatures during and after solidification must likewise be regulated according to conditions. Satisfactory results are obtained with temperatures ranging from 150° F. to 180° F. before the matrix has been removed from its base. After the matrix has been removed, higher temperatures can be used. Where the matrix is made of gelatinous material even lower temperatures may be necessary. The temperature should, of course, never be raised to a point where it will blister the phenolic resin or damage the matrix.

It will be appreciated by persons skilled in the art that beautiful, artistic material can be made by utilizing the principles of the invention in applying a synthetic resin layer or layers of any desired thickness, in which may be contained one or more coloring ingredients so as to give the layers the desired color. Phenolic resins may serve as a backing plate to receive the cold plasticizable phenolic resin which takes the impressions, which surfacing resin may be of such thickness and color as may be considered practicable or as will harmonize or contrast with the color of the base material. The thickness of such surfacing plastic may be as thin as  $\frac{1}{1000}$  of an inch or less, but may be much greater, depending upon the depth of the design to be reproduced.

When objects such as knife handles, medallions, ornaments, buttons, and numerous other articles are cut from a sheet or plate formed from molded material with contrasting colors, unusually attractive decorative effects can be obtained. The phenolic resin can also be further engraved, if desired, to bring out the base color in contrast with the color of the surface material.

It should be noted that the embossed designs illustrated in the drawing, although they may appear simple and crude, are in actual practice very beautifully and delicately embossed articles that defy accurate description. These fine engraving-like patterns cannot be obtained with ordinary thermoplastic methods without the expense of a number of specially made and engraved dies. With this invention the finest design may be very simply and economically made or reproduced without the necessity of such dies, and without the use of the extensive equipment heretofore required.

The design coating of the invention adheres to the backing with the utmost tenacity, owing to the fact that the resinous material of which it is made possesses a remarkable adhesive and binding strength.

While certain novel features of the invention have been disclosed and are pointed out in the annexed claims, it will be understood that various omissions, substitutions and changes may be made by those skilled in the art without departing from the spirit of the invention.

What we claim is:

1. The method of making decorative panels consisting of a fibrous baseboard coated with a cold moldable resin having a design embossed therein, which method comprises placing said baseboard on a flat bed, spreading thereover a relatively thin layer of cold moldable resinous compound, preparing a flexible matrix having the desired design embossed in cellulosic material, firmly progressively rolling said matrix into said resinous layer, mildly heating the assembly thus formed until the resinous compound sets, stripping the matrix therefrom, and again heating the embossed resinous layer on said fiberboard to effect final curing and hardening thereof.

40 2. The method of making decorative panels consisting of a baseboard coated with a cold moldable resin having a design embossed therein, which method comprises spreading a layer of cold moldable resinous compound over said baseboard, preparing a flexible matrix having the desired design embossed in cellulosic material, firmly rolling said matrix into said resinous layer, mildly heating the assembly thus formed until the resinous compound sets, and stripping the matrix therefrom.

55 3. The method of making decorative panels consisting of a relatively rigid fiberboard base sheet coated with a cold moldable resin of the phenolic or urea type having a design embossed therein, which method comprises spreading a layer of cold moldable phenolic or urea resin compound over said base sheet, preparing a flexible embossed cellulosic matrix, rolling the matrix into said resin, setting the resin, stripping the matrix therefrom, and heating said embossed resin compound fixed to said base sheet to effect final curing and hardening of said resin compound.

65 4. The method of making a multi-colored decorative panel comprising applying a coating of an accelerated cold moldable resin of selected color to the surface of a fibrous baseboard, preparing a cellulosic matrix having a design embossed therein, applying a cold moldable resin to the embossed surface of said matrix, removing excess resin from said embossed matrix so that the remaining resin will be contained in the depressed surfaces thereof only, pressure rolling said resin-coated matrix into adhering contact with said

first applied coating, mildly heating the assembly thus formed until the second applied resin coating has initially set, and afterwards stripping the matrix from said layer.

5. The method of making a multi-colored decorative panel comprising applying a coating of cold moldable resinous material to a relatively rigid fibrous base sheet, preparing a flexible celluloidic matrix having a design embossed thereon by areas depressed below the surface thereof, fill- 10

ing the depressed areas with a cold moldable resin having a different color than that of the first coating, setting the resin so deposited in said depressed areas, pressure rolling said treated matrix over said first coating to unite the cold moldable resin contained in said depressed areas to said first resinous coating, and afterwards stripping the matrix from said first layer.

OSWALD R. SCHULTZ.  
HENRY D. TUCKER.